

Oct. 20, 1925.

1,557,748

I. M. WASHINGTON

CONCRETE PLAQUE AND METHOD OF MAKING SAME

Filed Oct. 24, 1924



Fig. 1

Fig. 2



INVENTOR

Irene M. Washington  
BY *A. Van Pelt Smith*  
ATTORNEY

Patented Oct. 20, 1925.

1,557,748

# UNITED STATES PATENT OFFICE.

IRENE MARTHA WASHINGTON, OF BROOKLYN, NEW YORK.

CONCRETE PLAQUE AND METHOD OF MAKING SAME.

Application filed October 24, 1924. Serial No. 745,601.

To all whom it may concern:

Be it known that I, IRENE M. WASHINGTON, a citizen of the United States of America, residing at Brooklyn, city of New York, county of Kings, State of New York, have invented certain new and useful Improvements in Concrete Plaques and Methods of Making Same, of which the following is a specification.

10 My invention relates to the production of artistic plaques of cement mixtures which will present the effect of a painting on canvas or other given fabric having a characteristic surface, and reproduce any given 15 design. The best method at present known to me, for practising my invention is illustrated in the accompanying sheet of drawings in which:

Fig. 1 shows a sheet of canvas with a 20 simple design of a clover leaf appearing thereon.

Fig. 2 is a plan view of said sheet with bodies of cement applied to certain portions thereof in the process of forming the plaque, 25 and

Fig. 3 is a cross section on line 3—3 of Fig. 2.

Throughout the drawings like reference characters indicate like parts. 1 is a sheet 30 of canvas, burlap, or other material having a characteristic surface, a representation of which is to be reproduced in the cement plaque, and on which is marked the outline of the desired design, here shown as a clover leaf 2. The sheet bearing the design is supported on any suitable plane surface 3, and a frame 4 of the desired size and shape is placed on the sheet 1. 6, 6, represent masses 35 of hydraulic cement mixed with a green pigment placed on the sheet 1 over the sections of the design which are colored green, and 7, a mass of such cement mixed with a yellow pigment which extends over those portions of the design colored yellow. 8 40 represents a thicker backing preferably formed of concrete containing about three parts of sharp sand intimately mixed with hydraulic cement. 9 is a board on which the foregoing parts are assembled.

50 In operating according to my invention to make a cement plaque which shall reproduce the appearance or effect of a painting of said clover leaf or other design on canvas I mix pigments corresponding to the colors 55 to be reproduced with suitable masses of hydraulic cement, preferably neat, moisten

the masses with the proper proportion of water to combine with said cement when setting, and place the colored masses so produced on the canvas over the portions of the 60 design which are to have the same color in a layer of sufficient thickness to form an indestructible colored surface for the plaque. On this layer is then placed the 65 concrete backing which may be formed of hydraulic cement and sand of a thickness sufficient to produce, with the surface layer of colored cements, a plaque of the desired thickness and the entire mass is then allowed to set. The canvas is then stripped 70 off and the surface of the plaque will be found to present the characteristic appearance of a painting on canvas of the original design, being a replica of the canvas 75 surface in the selected colors.

Preferably the original layer of colored cement masses is allowed to partially set before the concrete backing is added. This is done to make sure that none of the concrete displaces the lower layer of colored 80 cement so as to appear on the face of the plaque. Preferably also pigments are used of mineral or other character which will not be soluble in the cement or affected by any of its constituents. This is to preserve 85 sharpness of outline in the design on the completed plaque.

While I have mentioned the use of hydraulic cement, obviously other cements might be used if plaques of fireproof or 90 other qualities characteristic of different varieties of cement are desired.

If it is desired to reproduce in the plaque the surface effect of any other material, such as cartridge paper, for instance, the 95 original design is outlined on a sheet of that material and the cement applied thereto as above described.

The result is an indestructible cement plaque which may be used for wall or other 100 decoration and will produce the effect of painting on canvas or any fabric having a characteristic texture or appearance.

Having described my invention, I claim:

1. The method of producing in a cement 105 plaque a reproduction of a design resembling a painting on any particular fabric which method comprises outlining the design on a sheet of such fabric, applying masses of cement colored to correspond to 110 different portions of said design on the corresponding areas of said fabric in a layer

of proper thickness, allowing the cement to set and finally stripping off said fabric from the face of the plaque so formed.

2. A method such as set out in claim 1 in which a backing of moist concrete is added to the layer of colored cement and allowed to set thereon.

3. A method such as set out in claim 1 in which the cement is colored by mixing there-with, while dry, pigments which are insoluble in any of the constituents of said cement when wet.

4. As a new article of manufacture, a cement plaque having a surface colored to 15 reproduce a particular design and reproducing the appearance of texture of a particular fabric.

5. As a new article of manufacture, a cement plaque reproducing the effect of a 20 painting on canvas having a surface representing a replica of a sheet of canvas composed of areas of cement mixed with different colored pigments.

6. As a new article of manufacture, a 25 plaque having a surface of hydraulic cement and a backing of concrete, said surface presenting a replica of a given fabric and containing mineral pigments mixed with the cement to reproduce a given design in colors,

whereby the effect of a painting of said design on said fabric is produced.

7. The method of producing in a cement plaque a reproduction of a design resembling a painting on any particular fabric which method comprises outlining the design on a sheet of such fabric, applying masses of moist hydraulic cement colored to correspond to different portions of said design on the corresponding areas of said fabric in a layer of proper thickness, allowing the cement to set and finally stripping off said fabric from the face of the plaque so formed.

8. The method of producing in a cement plaque a reproduction of a design resembling a painting on any particular fabric which method comprises outlining the design on a sheet of such fabric, applying masses of moist hydraulic cement colored to correspond to different portions of said design on the corresponding areas of said fabric in a layer of proper thickness, adding a backing layer of concrete containing hydraulic cement, allowing the cement to set and finally stripping off said fabric from 50 the face of the plaque so formed.

IRENE MARTHA WASHINGTON.